

## UNITED STATES PATENT OFFICE.

ROY D. HALL, OF EAST ORANGE, NEW JERSEY, ASSIGNOR TO WESTINGHOUSE LAMP COMPANY, A CORPORATION OF PENNSYLVANIA.

## FILAMENT.

No Drawing.

Application filed December 18, 1917. Serial No. 207,838.

*To all whom it may concern:*

Be it known that I, Roy D. Hall, a citizen of the United States, and a resident of East Orange, in the county of Essex and State of New Jersey, have invented a new and useful Improvement in Filaments, of which the following is a specification.

My invention relates to filaments for incandescent lamps, and more particularly to filaments made from highly refractory material, such as tungsten or equivalent material. The object of my invention is to produce a filamentary body composed of such constituents that when subjected to a predetermined heat treating schedule, the crystalline structure thereof may readily be given a characteristic formation.

It has been found that the crystalline structure of a metallic filament gives it certain inherent characteristics and that these characteristics are dependent upon such factors as the composition of the material comprising the filament, any treatment to which it has been subjected, etc. These characteristics manifest themselves by internal alterations of the filament under the influence of electric currents, and are usually designated by the terms "offsetting", "sagging", "non-sagging", etc. These properties may be more or less regulated by controlling the crystalline structure of the filament by the addition of certain ingredients to the tungsten during the process of forming the tungsten powder into a rod or ingot preparatory to swaging and drawing.

In accordance with the above facts, my invention contemplates the addition of certain auxiliary ingredients to the tungsten comprising a filamentary body, that will impart to the latter, such inherent characteristics as to make it highly responsive to a seasoning schedule designed to produce a given crystalline formation. I propose to use for the auxiliary ingredients a certain percentage of some oxygen containing compound, such as thoria or other rare earth metal oxide, alumina, etc. that is non-reducible in hydrogen and substantially non-volatile, and combine it with another oxide, such as silica, that becomes more or less volatile at high temperatures. I am aware that it has been common heretofore to use a considerable per cent of thorium oxide combined with tungsten as an offset resisting material and to a certain extent it has the function of controlling the subsequent crystallization of the filament, giving it an unusual grain fineness. However, I have discovered that when used in the percentages now common, namely from 3-7% by volume, it has a deleterious effect in retarding the formation of large over-lapping crystals which are necessary to prevent sagging of the filament, especially if of the coiled type. This retardation of the growth of large inter-lacing crystals, I believe, is directly traceable to the large percentage of thoria present. It is also true that when extremely large crystals are formed, other points of the lamp's efficiency are sacrificed, such as long life, etc. It would, therefore, appear that to produce a filament having a crystalline structure which would give non-sagging properties to the filament, it must be of such a composition as to be inherently capable of assuming a given structure when treated by a seasoning schedule. I have discovered that this may be accomplished by the mixture of a small percentage of a compound, such as thorium oxide or other rare earth metal oxide, aluminum oxide, etc., with a certain per cent of silica. Both the oxides of thorium or aluminum and silicon, are non-reducible in hydrogen and each have somewhat the same effect in retarding grain growth. However, the silica may be volatilized at a high temperature and in this way a considerable portion of it is freed from the tungsten during the formation of the tungsten powder into a filament. The method employed by the applicant in fabricating the tungsten into a filamentary body is the one described in the Coolidge Patent 1,082,933 of December 30, 1913. It would seem that a considerable quantity of these auxiliary materials is required at the start of the forming of the tungsten powder into a rod or ingot according to the processes practiced in producing ductile tungsten. This is perhaps, due to the fact that in the early stages the tungsten metal is worked at a very high temperature and this effects a more or less rapid volatilization of the silica. It, therefore, appears to be necessary that in order to obtain proper control of the inherent

properties desired to be imparted to the filament so as to make it susceptible to a predetermined seasoning schedule which will induce the formation of a given crystalline structure, it is necessary that a relatively large percentage of crystal growth resisting ingredients or materials be present initially. It is also a condition that one of these resisting materials be of such a composition that it may be gotten rid of later by volatilization or the like. The quantity of thoria and silica which I have mixed together and produces excellent results is from 2% to 7% by volume (.25% to 1% by weight) of silica and .1% to .4% by volume (.05% to .2% by weight) of thoria. In case it is desired to use alumina instead of thoria, equally satisfactory results may be obtained by adding 1% to 5% by volume (.2% to 1% by weight) of alumina with 2% to 7% by volume (.25% to 1% by weight) of silica. The use of this last mixture of auxiliary substances may be preferred since a certain percentage of aluminum is originally carried by the tungsten as an impurity and must be gotten rid of during the process of refinement in producing substantially pure tungsten. I find that when these percentages of the materials mentioned are used, a quality of wire is produced that is very responsive to a heat treating schedule such as disclosed by Harry H. Smith in an application filed Dec. 19, 1917, Serial No. 207,851, and results in the formation of a crystalline structure possessing substantially non-sagging properties.

While I have designated certain oxides of the rare earth metals as being one of the auxiliary substances added to tungsten in certain percentages, I do not wish to be limited to the specified quantities or metals mentioned, but my invention in its broadest aspect contemplates any metals having corresponding properties to those specified and bearing a similar percentage by volume to the tungsten to which they are added. The same is true for the other auxiliary ingredients mentioned, and I wish it understood that silica is simply one of the substances classifiable as volatile at high temperatures.

In the appended claims, I have defined certain substances as being "volatile" and "non-volatile" and I wish it understood that these terms as so used are to be considered with reference to the temperatures at which a refractory metal, such as tungsten, is worked. The same interpretation is desired to be given to the volatility at "high temperatures" of one of the substances specified, that is, volatile at a temperature which is high relative to those required for the working of tungsten.

What I claim is my invention is:

1. A filamentary body composed mainly

of tungsten or equivalent metal that at incandescence tends to sag when utilized as a conductor of electricity, and containing auxiliary ingredients capable of controlling the crystalline structure to produce a substantially non-sagging filament when subjected to a predetermined heat treatment. 70

2. A filamentary body composed mainly of tungsten or equivalent metal that at incandescence tends to sag and offset when utilized 75 as a conductor of electricity, and containing auxiliary ingredients which render the filamentary body inherently susceptible to a heat treating schedule designed to produce a crystalline formation resistant to sagging 80 and offsetting.

3. A filamentary body composed primarily of tungsten and containing a non-metallic material capable of promoting crystal growth resistant to sagging when 85 said body is converted into a filament and heated to elevated temperatures.

4. A filamentary body composed primarily of tungsten and containing a material capable of exerting an influence to promote 90 the development of large crystals having such size and contour as to prevent substantial sagging or substantial offsetting when converted into a filament and heated to elevated temperatures. 95

5. A filamentary body composed of tungsten or equivalent material that tends to sag when utilized as a conductor of electricity and containing ingredients capable of promoting crystal growth in said body when 100 converted into a filament and heated to elevated temperatures.

6. A filamentary body composed of tungsten or equivalent material that tends to sag and offset when utilized as a conductor of electricity and containing ingredients capable of promoting crystal growth resistant to sagging and offsetting. 105

7. A filamentary body composed primarily of tungsten and containing a material which volatilizes mainly at high temperatures and is capable of directing crystal growth. 110

8. A filamentary body composed primarily of tungsten and containing a material which volatilizes mainly at high temperatures and another material substantially non-volatile at such temperatures, said materials being capable of directing the crystalline growth of said body. 115

9. A filamentary body composed primarily of tungsten and having intimately associated therewith a non-metallic substance capable of promoting crystal growth. 120

10. A filamentary body composed primarily of tungsten and having intimately associated therewith a compound or compounds containing silicon and oxygen and capable of directing crystal growth in said body. 125

11. A filamentary body composed primarily of tungsten and having intimately associated therewith a compound or compounds containing silicon, thorium and oxygen. .1% to .4% by volume (.05% to .2% by weight) of thoria. 40
12. A filamentary body composed primarily of tungsten and having intimately associated therewith a compound or compounds containing silicon and oxygen with 10 a small percentage of a substantially non-volatile compound and capable of directing crystal growth in said body. 17. The method of producing a filamentary body capable of having imparted thereto upon heat-treatment, a crystalline formation resistant to sagging and offsetting, which comprises intimately mixing tungsten or an equivalent metal and auxiliary ingredients capable of directing the crystalline structure of the tungsten, one of said auxiliary ingredients being substantially non-volatile and another of said ingredients being volatile only at high temperatures, and thereafter forming a filamentary body therefrom in accordance with the method herein set forth. 45
13. A filamentary body composed primarily of tungsten and having intimately associated therewith a compound or compounds containing a substance which volatilizes at high temperatures and one which is substantially non-volatile at such temperatures and capable of directing crystal growth in said body. 18. The method of producing a filamentary body capable of having imparted thereto upon heat-treatment, a crystalline formation resistant to sagging and offsetting, which comprises intimately mixing powdered tungsten, thoria and a compound 50 or compounds containing silicon and oxygen, and forming a filamentary body therefrom in accordance with the method herein set forth. 55
14. A filamentary body composed primarily of tungsten and having intimately associated therewith a compound or compounds containing ingredients some of which are volatile at high temperatures and others non-volatile at such temperatures and capable of directing crystal growth in said body. 19. The method of producing a filamentary body capable of having imparted thereto upon heat-treatment, a crystalline formation resistant to sagging and offsetting, which comprises mixing powdered tungsten, thoria and silica and thereafter 60 forming a filamentary body in accordance with the method herein set forth. 65
15. A filamentary body composed primarily of tungsten to which has been added during its manufacture from 2% to 7% by volume (.25% to 1% by weight) of silica and 1% to 5% by volume (.2% to 1% by weight) of alumina. 30
16. A filamentary body composed primarily of tungsten to which has been added during its manufacture from 2% to 7% by volume (.25% to 1% by weight) of silica and 35
- In testimony whereof, I have hereunto subscribed my name this 5th day of Dec., 1917.

ROY D. HALL.